

# UNITED STATES PATENT OFFICE.

JOSEPH HURYCH, OF BROOKLYN, NEW YORK.

## ALLOY.

SPECIFICATION forming part of Letters Patent No. 390,972, dated October 9, 1888.

Application filed April 5, 1888. Serial No. 269,762. (No specimens.)

*To all whom it may concern:*

Be it known that I, JOSEPH HURYCH, of Brooklyn, in the county of Kings and State of New York, have invented certain new and useful Improvements in Alloys, of which the following is a specification.

This invention relates to an improved alloy of zinc, lead, tin, and antimony, which is to be used for wash-tubs, bath-tubs, sinks, journal bearings, and other articles; and the invention consists of an alloy composed of ninety pounds of zinc, four pounds of lead, three pounds of tin, and two pounds of antimony.

My alloy is made in the following manner: For every one hundred pounds of the same, 15 ninety pounds of zinc, four pounds of lead, three pounds of tin, and two pounds of antimony are used. These metals are melted in

separate parts and united in the mold, they being poured into the same in the order of 20 their higher specific gravities, whereby the proper union of the metals into a strong and durable alloy is obtained.

Having thus described my invention, I claim as new and desire to secure by Letters Patent— 25

An alloy composed of ninety pounds of zinc, four pounds of lead, three pounds of tin, and two pounds of antimony, substantially as described.

In testimony that I claim the foregoing as my 30 invention I have signed my name in presence of two subscribing witnesses.

JOSEPH HURYCH.

Witnesses:

PAUL GOEPEL,  
CARL KARP.